

## UNITED STATES PATENT OFFICE

FRED J. CROLIUS AND RUDOLPH W. STULER, OF PITTSBURGH, PENNSYLVANIA, AS-  
SIGNORS TO STAINLESS STEEL CORPORATION, A CORPORATION OF DELAWARE

## TREATMENT OF METAL

No Drawing.

Application filed November 12, 1930. Serial No. 495,282.

It has been proposed to treat molten metal, particularly iron or steel or alloys thereof, with a sudden shock or mechanical disturbance to obtain especial benefits in the characteristics of the final product when cast or cooled. It has been proposed to procure this sudden shock by chemical means, that is an explosive material introduced into the bath of the molten metal.

10 It is the purpose of the present invention to produce a sudden shock or a series of sudden shocks in a bath of molten metal and thus produce all of the benefits incident thereto without the injection of any explosive or other chemicals into the metal. Among other things this eliminates the possibility of there being any remnant of the explosive in the final product. Since generally there is no desirability of having any portion of 20 the explosive material remain in the metal its complete exclusion is desirable. Indeed, it may be that the presence of the explosive material is undesirable and deleterious in the final product.

25 It has been found that an improved product may be produced by giving to the molten metal by electric means a shock sufficient to produce the desired results. This shock but avoids a real explosion and so avoids the 30 possibility of accidents due to high pressures or to spattering or distribution of hot metal outside its container.

35 When it is desired to carry out the present invention iron, steel or alloys thereof may be produced in the usual way in the usual furnaces and then the molten metal may be introduced into an electric furnace and the shock produced by suddenly turning on the full current to affect the metal bath in the furnace.

40 It may be more desirable, however, to carry out the manufacture of the metal or at least its alloying in an electric furnace and produce the desired shock by turning off the current and allowing the metal to become quiescent and then suddenly turning on the current to produce the shock. This may be 45 safely done either in a closed or an open furnace without the liability of throwing out

the metal as might occur if there were an internal explosion.

To the carrying out of the present invention is especially adapted the Ajax type of crucible high frequency electric furnace, sometimes referred to as a coreless electric furnace. A ladle type Ajax furnace may be employed to bring a melt of approximately 300 pounds of alloy steel to nearly the final addition point. For instance the carbon steel will be melted, the lime slag will have boiled, risen, and the manganese may have been added and the heat apparently completed or "made." The temperature at this point may be approximately 2850° F. The current in the furnace is abruptly cut off. Then current is suddenly turned on and the full force of say 150 kw. of alternating current is pressed into the furnace at a frequency of between 1000 and 2000 cycles. Incidentally the mass is agitated and boils, with increasing temperature and violently increased circulation.

Every indication of severe shock is observed. Slag previously occluded is freed and rapidly agglomerates on the surface. Gases are freely and profusely liberated. The metal becomes remarkably fluid and when cast into ingots shows a denser structure and a better surface than corresponding alloys poured when "made" and not submitted to the shock. These beneficial characteristics continue throughout the rolling or other treatment of the metal into its desired finished shape.

Sometimes it is desirable after turning off the current to add to the molten batch further slag beneficiators or further alloying materials or both. This generally should be done while the current is turned off and before the mass is given the shock by suddenly turning on the current.

The procedure indicated produces good results but it may be desirable to submit the metal to a succession of shocks in which event the steps of shutting off the current and again suddenly turning on the current may be repeated a suitable number of times.

The details here indicated are not essential to the invention and those versed in the art

will understand that it may be applied in other ways and be employed as a step in the manufacture of various steels, irons and alloys. The other steps of such manufacture may be adopted, adjusted and varied to suit the needs or desires of the operator.

5 We claim as our invention:

- 10 1. The process of preparing metal in high frequency electric furnaces which comprises subjecting a molten bath of the metal to a sudden shock by suddenly turning into the furnace the full force of the alternating current.
- 15 2. The process of preparing metal comprising melting and treating it in a high frequency electric furnace, shutting off the electric current, and turning on the electric current to give a sudden shock to the metal.
- 20 3. The process of preparing metal comprising heating the metal in a high frequency electric furnace to the final addition point at about 2850° F., turning off the current, suddenly turning on a current of 150 kw. with a frequency of between 1000 and 2000 cycles.
- 25 4. The process of preparing metal comprising heating the metal in a high frequency electric furnace to the final addition point, shutting off the current, adding elements desired, and suddenly shocking the metal by turning on the current.
- 30 5. The step in preparing metals comprising shocking a molten bath of the metal in a high frequency electric furnace by suddenly subjecting it to sufficient electric current to shock the bath.
- 35 6. The step in preparing metal comprising repeatedly shocking a molten bath of the metal in a high frequency electric furnace by repeatedly suddenly subjecting it to sufficient electric current to shock the bath.
- 40 7. The process of preparing metal comprising heating the metal in a high frequency electric furnace to the final addition point, shutting off the current, adding elements desired, and suddenly subjecting it to a sufficient electric current to shock the bath a plurality of times.

F. J. CROLIUS.  
RUDOLPH W. STULER.